

(No Model.)

2 Sheets—Sheet 1.

T. T. ABBOT.

ART OF MANUFACTURING COTTON YARN.

No. 317,608.

Patented May 12, 1885.



FIG. 1.



FIG. 2.



WITNESSES:

Avery F. Cushman

William A. Saugert

INVENTOR:

Theodore J. Abbot  
by Elmer P. Horne, Atty.

(No Model.)

2 Sheets—Sheet 2.

T. T. ABBOT.

ART OF MANUFACTURING COTTON YARN.

No. 317,608.

Patented May 12, 1885.



FIG. 4.



FIG. 8.



FIG. 2.



FIG. 8.



FIG. 6.

WITNESSES:

Amy F. Lichman

William A. Gray

INVENTOR:

Theodore J. Abbot

Elmer P. Stor

att'y.

# UNITED STATES PATENT OFFICE.

THEODORE T. ABBOT, OF LUNENBURG, ASSIGNOR TO THE ABBOT SPINNER COMPANY, OF BOSTON, MASSACHUSETTS.

## ART OF MANUFACTURING COTTON YARN.

SPECIFICATION forming part of Letters Patent No. 317,608, dated May 12, 1885.

Application filed November 8, 1884. (No model.)

*To all whom it may concern:*

Be it known that I, THEODORE THOMAS ABBOT, of the town of Lunenburg, county of Worcester, and State of Massachusetts, have 5 invented a new and Improved Process of Spinning Cotton Yarn, of which the following is a specification.

In the ordinary process of spinning cotton it is, after being blown and cleaned and made 10 into "laps" or "fleeces," as they are sometimes called, submitted to the action of carding-engines, and there carded and converted finally into a sliver, which is a tape-like product composed of filaments of cotton held slightly together in some way, probably by a slight interlocking of the finer filaments. The sliver is then in drawing-frames subjected to the operation of drawing and doubling with a view 15 to evening it and bringing it to a condition suitable for the production of an even, firm, and uniform yarn. When the sliver, which at this stage is usually termed "drawing," leaves the last of these frames and is received in a can, it has no twist in it, but is still a tape or ribbon 20 with the fibers more nearly parallel to its length than when it came from the carding-engine. I say "it has no twist in it;" but this is not the exact truth, as the cans into which the slivers are received from the finishing-cards 25 or the first drawing-head, (viz., that working in connection with the carding-engine,) or some or all of the drawing-frames, have usually a slow revolving motion, and this motion puts one turn into the sliver for each revolution 30 of the can. This twist is, however, almost imperceptible. The next step is to convert the "drawing," so called, into roving. This is effected by again submitting it to the action of drawing-rollers which are in the 35 same frame and combined with spindles and fliers, and in such frame the sliver is again doubled or trebled and drawn, or merely drawn, and finally twisted by spindles and fliers and wound upon bobbins. In this twisted state it is in a second machine wound off 40 from the bobbins and again doubled and drawn, or merely drawn, and again twisted by spindles and fliers and wound upon other bobbins. These last bobbins are usually carried to a 45 third machine, where similar operations are performed, and the material becomes what is

called "fine roving." Sometimes a fourth machine of similar character is employed when finer numbers are required. These four machines, to the first of which the slivers are 55 supplied, each draw and twist the material, and the material after it comes from the first of the machines is known as "roving." These machines are sometimes called "speeders," or, respectively, the "slubber," the "intermediate," the "fine roving," and the "jack-frame." The final step is to convert the roving into yarn. To this end the fine rovings from the last machine of the series, while wound upon bobbins, are next submitted to 60 the operation of mules, thrusters, or ring spinning frames, where they are spun into yarn, and in the ring-spinning frames, the thrusters, and usually the mules, the roving is further drawn by drawing-rollers before it is spun. 65 Such is the ordinary process of spinning cotton yarn. Its practice necessitates the employment of a large number of machines, which not only are both costly in the first instance and a source of continuing expense, but require for their use a large amount of room 70 in the factory or mill. Furthermore, it involves frequent handling of the material, which is objectionable, and the twisting incident to the conversion of the sliver into 75 roving impairs the strength of the yarn, and is apt to render it harsh and kinky. With a view to obviating these disadvantages various expedients have heretofore been suggested. It has been proposed, for instance, 80 to combine in one machine a carding-engine, rub-aprons or rollers for condensing and putting into shape and conveying the material as it is stripped from the carding-cylinder, and spinning devices for spinning the same 85 into yarn, the material passing continuously from the card through the rub-aprons or the rollers to the spinning devices. This plan, however, contemplates the splitting of the cotton lap, which is difficult, if not impracticable, and does not provide for evening the 90 silver. It has also been attempted, with what success I do not know, to consolidate the three or four machines usually employed to convert sliver into roving by using in a single machine 95 a number of pairs of drawing-rollers in series, in combination with either stationary or re-

volving trumpets or condensers between the sets of rollers, in order to compact or condense the sliver, and with spindles and fliers at the end of the series of drawing-rollers and trumpets, the machine thus organized and when working producing a roving wound upon bobbins similar to that which is usually manufactured by the fine roving or the jack-frame, the fineness of the roving depending upon the 10 number of sets of drawing-rollers employed. This plan is meritorious in that it makes one machine do the work of the three or four ordinarily employed for the purpose; but it still involves the twisting of the fiber prior to the 15 ultimate spinning operation, and the product is distinctively not yarn, but roving made up of twisted fibers, which must be drawn again and ultimately twisted in the mule, throste, or ring-spinning frame, by which it 20 is spun into yarn.

Manifestly it would be of great advantage to avoid the use of machinery for converting the sliver into roving, and to maintain the sliver in untwisted state until it receives the 25 ultimate twist at the time it is converted into yarn. This result is accomplished by my invention.

I have discovered that cotton fiber may be spun into yarn by first bringing it to the condition of sliver, subjecting it to the drawing and doubling operation for the purpose of evening it, and then conducting it directly to the spinning-frame, in which it is spun into finished yarn. I thus avoid the intermediate 30 step of converting the sliver into roving, and neither twist the fibers nor wind them upon bobbins prior to the time when the ultimate twist is given to them to make finished 35 yarn.

40 In the preferred way of carrying out my invention I take ordinary sliver furnished by carding-engines and draw and double these slivers in the ordinary way. These slivers thus drawn have no practical twist in them, although they may have such slight twist as is produced by the ordinary revolutions of the 45 cans into which the slivers are received. In fact, I take such sliver as is usually furnished to the slubber and convert it directly in a single machine into finished yarn. In this single machine the sliver is drawn, compacted, or 50 condensed, and spun directly into yarn, thus saving the use of the slubber, the intermediate, the fine roving, and the jack-frame, and 55 putting no twist (except that produced by the revolution of the cans) into the sliver until it receives the final twist on the spindles.

In carrying out my process I neither make roving as an intermediate step of a process 60 nor double nor draw roving, and I find that by my process I produce a yarn of increased strength, which is soft and fluffy and much similar to the yarn which is spun upon the mules in the usual manner.

65 To better enable others skilled in the art to understand and use my invention, I have illustrated in the accompanying drawings a ma-

chine, also of my invention, adapted to be used in the practice of the process. I wish to be understood, however, that I do not here 70 claim said machine, but that the same is made the subject of separate Letters Patent of even date herewith.

Figure 1 is an end view of the machine. Fig. 2 is a front elevation thereof with the center 75 portion broken away to bring the ends nearer together. Fig. 3 is a front elevation of the drawing-rollers with the center portion broken away, as in in the last preceding figure. Fig. 4 is an end elevation of the drawing-rollers 80 and their supporting-frame, showing the gearing at that end for driving the said rollers, the bracket or stand which furnishes the bearings for the intermediate gear-wheels, or some of them, being broken away. Fig. 5 is a like 85 elevation of the other end of the frame and rollers with the bracket or stand at that end broken away, as in the last preceding figure. Fig. 6 is a cross-section on line  $x-x$  of Fig. 3. Fig. 7 is a cross-section on line  $y-y$  of Fig. 3. 90 Fig. 8 is a top view of the drawing-rollers, their driving-gearing, and supporting-frame, the center portion of the rollers being broken away. In that portion of the figure to the right of the break the upper rollers are removed to 95 expose to view the lower or fluted rollers and the trumpets. Fig. 9 is a section on line  $z-z$ , Fig. 8.

There is shown in the drawings a machine provided with several sets of drawing-rollers, 100 the slivers passing through the grip of six pairs of drawing-rollers of each set. These rollers may be of any known construction and caused to revolve by any known kind of machinery, and the upper may be pressed upon 105 the lower rollers in any known way. Moreover, I do not confine myself to any precise number of pairs of rollers, nor to any precise speed of revolution thereof, nor to any precise relation of the speed of one roller to that 110 of its successor in the series; but I prefer to revolve the third pair of rollers at the same or at about the same speed as the second pair, and the fifth pair at about the same speed as the fourth pair, and so on in succession when 115 more than six pairs are used, the fiber being thus drawn between the first and second and the third and fourth and the fifth and sixth pairs of rollers. The slivers may be doubled and drawn by these rollers; but I prefer merely 120 to draw them.

In spinning No. 20 yarn, for instance, I use sliver weighing sixty grains to the yard, and run the first pair of rollers,  $a-a'$ , with a surface-speed of two and twenty-two one-hundredths inches per minute; the second pair,  $b-b'$ , with a surface-speed of seven and ninety-two one-hundredths inches per minute; the third pair,  $c-c'$ , at the same speed as the second pair,  $b-b'$ ; the fourth pair at a surface-speed which is forty-eight and thirty-three one-hundredths inches per minute; the fifth pair,  $e-e'$ , at the same speed as the fourth pair, and the sixth pair at a surface-speed of three 130

hundred and fourteen inches per minute. At these revolutions of the rollers I run the spindles, according to the number of turns to the inch desired in the finished yarn, at from six 5 thousand to seven thousand revolutions per minute. These speeds may of course be varied either absolutely or proportionately for the same number of yarn or for different numbers of yarn and for different weights of sliver; but the 10 experienced spinner will know how to vary the speeds properly or even the number of pairs of rollers, according to the required extent of elongation or drawing of the sliver before it is spun, after reading the rule I have given for 15 No. 20 yarn from sliver weighing sixty grains to the yard. I cannot draw the sliver to the extent required without using trumpets to condense or compact the sliver as it is being drawn, the trumpets serving to gather the 20 out-lying or outwardly-projecting fibers into the body of the sliver; and I prefer to use with six pairs of rollers three trumpets, *g h i*, for each sliver, the first trumpet acting upon the sliver as it enters the frame, the second applied 25 between the second and third pairs of rollers, and the third between the fourth and fifth pairs; but I intend to use a greater or less number of trumpets. These trumpets I prefer to make stationary or non-revolving, but 30 they may be of any usual construction.

The sliver *t*, delivered by the last pair of drawing-rollers, is furnished to spindles provided with rings and travelers, (shown at *k k*.) and spun by them, as usual, except that the yarn receives 35 its whole necessary twist by means of these spindles, the spindles spinning the yarn from drawn and doubled sliver, and not from drawn and doubled roving, as usual. These spindles, rings, travelers, and the mechanism for 40 driving them may be of any usual construction.

The sliver to be drawn and spun in my machine is contained in cans *m m*, by preference arranged in a double tier one above the other, and supported above the drawing-rollers on a can-stand, *o o*, and the sliver is lifted out of 45 these cans by rollers *n n*, over which the sliver passes, as usual; and I prefer to make the machines double, as shown in the drawings—that is, with two complete sets of cans, drawing-rollers, trumpets, ring-spindles, and their 50 accessories.

In the operation of the machine the sliver is taken from the cans, drawn by the rollers, compacted or condensed by the trumpets, and finally spun into yarn by the spindles. 55

I claim as of my own invention—

1. The described process of making cotton yarn, consisting in bringing the cotton fiber to the condition of sliver and drawing and doubling the sliver for the purpose of evening it, 60 then further drawing and compacting or condensing without twisting the sliver thus prepared until it is reduced to the attenuated form requisite to allow it to be spun directly into yarn, and finally spinning said attenuated sliver directly into finished yarn, as contradistinguished from roving, the whole process being substantially such as hereinbefore set forth. 65

2. The method of making yarn directly from 70 sliver, consisting in taking sliver in the condition of that usually furnished to slubbers and drawing, compacting, and spinning the same, substantially as described, no twist being imparted to such sliver until it is ultimately spun into yarn. 75

THEODORE T. ABBOT.

Witnesses:

I. H. RUSSELL,  
G. D. BRAMAN.